

Jan. 6, 1925.

1,521,717

W. A. SCHMIDT

## PROCESS FOR STRAIGHTENING RIFLE BARREL FORGINGS

Filed Dec. 13, 1918



## UNITED STATES PATENT OFFICE.

WILHELM A. SCHMIDT, OF ILION, NEW YORK, ASSIGNOR, BY MESNE ASSIGNMENTS, TO REMINGTON ARMS COMPANY, INC., OF NEW YORK, N. Y., A CORPORATION OF DELAWARE.

## PROCESS FOR STRAIGHTENING RIFLE-BARREL FORGINGS.

Application filed December 13, 1918. Serial No. 266,620.

To all whom it may concern:

Be it known that I, WILHELM A. SCHMIDT, a citizen of the United States, residing at Ilion, in the county of Herkimer and State

5 of New York, have invented a certain new and useful Improved Process for Straightening Rifle-Barrel Forgings, of which the following is a specification.

This invention relates to a process for 10 straightening rifle barrel forgings and for relieving internal stresses and strains from such forgings.

One object of the invention is to produce a rifle barrel or other similar article at a 15 lower cost than by methods heretofore used.

Another object is to produce a barrel from 20 which internal strains are practically or entirely absent so that the barrel will not warp out of true after use as is sometimes the case in barrels made by the processes heretofore used.

Other objects are to improve generally former methods for constructing rifle barrels and other like articles whereby I am 25 enabled to make a better article at a lower cost.

I attain these objects by the improved process hereinafter fully described and claimed.

30 The single sheet of drawings annexed hereto shows an actual stress-strain diagram of a hot steel rod under tension and illustrates graphically the effect of tension on internal stresses and strains.

35 The manufacture of rifle barrels as heretofore practiced was effected substantially as follows:

The rifle barrel forging was formed 40 roughly from heavy round stock by rolling or forging under a hammer. A large percentage of these forgings were found to be curved by these operations and needed straightening. This was partially accomplished under a long die while the metal was hot followed by a cold straightening 45 operation before machining. Where cold straightening was necessary the bending was necessarily carried far enough to strain the outer fibers beyond the elastic limit. When 50 the bending force was removed those fibers

which had been strained beyond the elastic limit set up stresses in the opposite direction, which held the forging substantially straight.

These forgings subsequently underwent a 55 number of machining operations. Between these machining operations it was found necessary to inspect and straighten the barrels a number of times.

It is well known that the reduction of 60 metal by rolling or forging will set up internal stresses and strains in the resulting forging, i. e., in any transverse section of the forging certain fibers will be in compression while others are in tension. These 65 strains are irregularly distributed throughout the metal but necessarily are so disposed on every transverse section that the sum of the forces resulting from the compression strains is equal to the sum of the forces due 70 to the tension strains and so disposed relative to each other that their respective turning moments about any axis are equal and opposite. This will be the case whether the forging happens to be straight or crooked. 75

If the forging is not straight it will require straightening. The result of this will be to further increase the internal strains and to further decrease the homogeneity of the metal.

80 It was found that, when forgings made by this old method were machined, the resulting barrel was out of true. The removal of the outside metal had destroyed the delicate balance of complex internal tension and 85 compression stresses, together with their corresponding turning moments, so that a readjustment was necessary, one result of which was the warping of the barrel.

It was necessary to straighten these barrels, but the next machining operation 90 would again destroy the balance of internal stresses and necessitate further straightening. A number of alternate machining and straightening operations were necessary 95 to complete the barrel, but even the finished barrel was straight merely because the internal stresses happened to be balanced when the barrel was straight and it was found that the many temperature changes, 100

vibrations and intermittent stresses incident to the firing of the gun would in time disturb this balanced condition with the result that permanent warping of the barrel took place.

It is a fact well known to shooters that if a number of shots are fired from some rifles as heretofore made, the later shots are likely to be grouped some distance off of the target and that the sights will have to be reset after a certain number of shots. The reason for this is that the metal of such barrels is not homogeneous and that therefore, the expansion due to heating is not uniform. For this reason such a barrel may be perfectly straight when cold and still be crooked after a few shots.

Another well known difficulty was that barrels which appeared to be perfectly straight on final inspection would frequently not shoot accurately when tested in the gallery. The reason for this is not definitely known but the explanation sometimes advanced is that the inaccuracy is due to internal strains in the barrel. When a high power rifle is shot the barrel is violently "whipped." This "whip" is a transverse vibration and throws the barrel into waves similar to the waves which can be sent along a rope by suddenly moving it transversely at one end. If a barrel is normally under internal stresses these waves are irregular or of variable wave length or amplitude with the result that the shots are unaccountably scattered.

Whatever the cause of such erratic results may be, it has been found from tests of many thousands of barrels manufactured according to my present process that rejections from such causes have been much reduced.

These many difficulties have been practically overcome by my present invention.

In my process the forgings are formed by rolling as formerly. Then immediately after rolling and while the forging is still at a red heat the forging is placed in a stretching machine and elongated slightly beyond its elastic limit. This stretching operation is performed in a special machine which forms the subject of Patent #1,367,-099, February 1, 1921, but it is evident that any suitable machine may be used for this purpose.

The effect of this stretching is two-fold; it straightens the forging, but, what is of greater importance, it relieves it of internal strains. This forging is now permitted to cool and is ready for the necessary machining operations.

If the forging is not of a uniform cross section, for example, if it has an enlarged breech end, it may be necessary to true up the larger portion under a drop hammer. The reason for this is, of course, that the stress exerted in the larger section will be

much less than in the section of smaller area and will therefore not exceed the elastic limit.

After this the barrel is alternately machined and inspected for straightness. It has been found in practice that a barrel forging which has been treated according to my new process will seldom need straightening between these machining operations and many of the barrels pass this large number of inspections without requiring a single cold straightening.

Now we will consider the effect of the stretching operation upon the physical condition of the metal. The drawing illustrates the actual stress strain curve of a hot forging, the stress being laid off on the line OY while the corresponding strains are laid off on the line OX.

When the tensile stress is applied to the barrel the strain is found to be proportional to the stress applied, until the elastic limit is reached, which is in accordance with Hook's law. This part of the operation is graphically represented by the line OA. Beyond the elastic limit strain increases faster than the stress as shown by the line AB. At the point B the stress strain curve is horizontal. In the use of my process the load and consequently the stress is removed at a point somewhat beyond the elastic limit. It has been found that in most cases the load may be removed at C, i. e., at 1.5 per cent elongation or that the stretching may be carried somewhat beyond the point B if the forging is at the proper temperature. The elastic limit having been exceeded the forging retains a permanent set.

Now let us see what has happened to those fibers which were under stress before the load was applied. The line O'', A'', B'' represents the effect of tension on a fiber normally under a tension, represented by O, O''. Since all the fibers presumably have the same modulus of elasticity the line O'', A'' will be parallel to the line O, A. From A'' to B'' the curve will be of the same shape as the curve AB.

The line O', A', B' represents the effect of tension on a fiber normally in compression. It will be noticed that the line O', A' does not cross the zero line OX until the tensile stress represented by the line O' O has been applied. The elastic limit is reached at A' and the curve becomes horizontal at B'. It will be noted that the three curves shown are identical in shape but slightly transposed in a horizontal direction. It will also be noted that while there is a considerable vertical distance between the curves below the elastic limit, that this is gradually decreased and becomes zero where the curves are horizontal. The curve E, F, G shows graphically the rapid decrease of the vertical distance between the

curves and indicates the rapidity with which difference in stress disappears as the stretching goes on. Until the elastic limit is reached no decrease takes place and the curve 5 is horizontal for about the first  $\frac{1}{2}\%$  of elongation but then it drops rapidly so that at 1% elongation the difference of stress has dropped to less than one-eighth of its original value and at the point C the difference 10 in stress is only about one-fourteenth of the original difference.

It is therefore evident that whatever the initial condition of any fiber, whether it be 15 at rest or under more or less tensile or compressive stress, when the forging is stretched to approximately the point B all fibers will be strained the same distance and will be under the same stress. When the load is entirely removed all of the fibers are at rest, 20 there are neither compressive nor tensile stresses. All internal stresses have been relieved and when the forging is subsequently machined, the removal of the metal will not disturb the balance of the internal stresses 25 as in forgings which have not been so treated. If the stress is removed before the point B is reached some slight internal stresses may still persist but they are too small to be of practical importance and it 30 has been found that very good results are obtained if the stress is removed at or above approximately the point C. It is of course understood that the stretching operation is carried out when the barrel is at the proper 35 temperature so as not to injuriously affect the physical properties of the metal. The particular temperature suitable for this purpose depends upon the nature of the metal or alloy of the barrel. For steel a dull red heat will give good results. A 40 much lower temperature will be satisfactory for the more ductile metals.

It will be seen therefore that I have invented a process which will at one operation 45 straighten barrel or other forgings and relieve the internal stresses set up by prior operations, which taken together with any subsequent machining steps will produce a barrel not only quicker and cheaper but also 50 much better in that it will not be inclined to permanently warp out of true as is the case in barrels constructed by any other process. Barrels made by this process will not temporarily warp out of true after a few shots 55 as so often happens with barrels straightened by bending or without stretching as required by my present process. Another effect, also referred to above, is that such barrels will shoot more accurately because their 60 vibration whip is uniform.

Another great advantage which this method of straightening has resulted in is the high degree of symmetry of mass around the axis throughout the length of the forging 65 which results in obtaining a straighter

hole in drilling. This is due to the fact that the drilling operation is performed by rotating the forging at a high rate of speed while the drill remains stationary, and owing to the homogeneity of the metal produced by my process there is practically no tendency of the forging to become displaced by bending transversely during the process of drilling as is the case with forgings which are not balanced relative to the axis of rotation, due to centrifugal action which tends to result in the drill being forced from the center of the barrel during the drilling operation. It has also been found by actual test that forgings stretched in this way are 70 somewhat improved in their physical properties. The elastic limit and the percentage of elongation are somewhat increased.

While I have described my invention as used in connection with the manufacture of 75 rifle barrels it is of course obvious that it is also applicable to the manufacture of other articles, but probably all of its functions will be realized only when used in manufacturing gun barrels. 80

However, what I regard as my invention and desire to protect by Letters Patent of the United States, is:—

1. The process of producing straight forgings which consists in first rolling the 95 forging definitely to shape and then straightening it by stretching the forging beyond the elastic limit while at a temperature at which the stretching will not injuriously affect the physical properties of the 100 metal.

2. The process of producing straight forgings which consists in first rolling the forging definitely to shape and then straightening it by stretching the forging beyond the 105 elastic limit while at a temperature at which the stretching will not injuriously affect the physical properties of the metal, cooling the forging and machining it.

3. The process of producing straight forgings having an enlarged end which consists in first rolling the forging to shape, straightening the enlarged end portion under a hammer, and then straightening the remaining portion by stretching the forging definitely beyond the elastic limit while at a 115 temperature at which the stretching will not injuriously affect the physical properties of the metal.

4. The process of producing straight forgings having an enlarged end which consists in straightening the enlarged end portion under a hammer, and straightening the remaining portion by stretching the forging definitely beyond the elastic limit while at a 120 temperature at which the stretching will not injuriously affect the physical properties of the metal.

5. The process of producing straight forgings having an enlarged end which consists 130

- in first rolling the forging to shape, straightening the enlarged end portion under a hammer, and then straightening the remaining portion by stretching the forging definitely beyond the elastic limit while at a temperature at which the stretching will not injuriously affect the physical properties of the metal, cooling the forging and machining it.
6. The process of producing straight forgings, having an enlarged end which consists in straightening the enlarged end portion under a hammer, and then straightening the remaining portion by stretching the forging definitely beyond the elastic limit while at a temperature at which the stretching will not injuriously affect the physical properties of the metal, cooling the forging and machining it.
- 10 7. The process of straightening a rifle barrel forging and relieving it of internal strains which consists in elongating the forging beyond its elastic limit while hot to a point where the stress-strain curve is substantially horizontal.
- 15 8. The process of straightening a gun barrel forging and relieving it of internal strains which consists in elongating the forging beyond its elastic limit while hot to a point where all fibers which were normally in compression have been strained to a point where their elongations is continued without an increase in total stress.
- 20 9. The process of straightening a rifle bar-

rel forging and relieving it of internal strains which consists in elongating the forging beyond its elastic limit while hot to a point where all fibers have been strained to a point where their elongation is continued without an increase in total stress.

10. The process of straightening a gun barrel forging and relieving it of internal strains which consists in elongating the forging to a point beyond its elastic limit and not exceeding the point where its elongation is continued without an increase in stress.

11. The process of straightening a gun barrel forging and relieving it of internal strains which consists in elongating the forging to point definitely beyond its elastic limit while at a dull red heat.

12. The process of straightening a gun barrel forging and relieving it of internal strains which consists in heating the forging to a dull red heat and then elongating the forging beyond its elastic limit while hot to a point where all fibers have been strained to a point where their elongation is continued without an increase in total stress.

13. The process of straightening a rifle barrel forging and relieving it of internal strains which consists in elongating the forging beyond its elastic limit while at a dull red heat to a point where the stress-strain curve is substantially horizontal.

In testimony whereof I affix my signature.  
WILHELM A. SCHMIDT.